

Patented Aug. 3, 1926.

1,594,853

# UNITED STATES PATENT OFFICE.

JULIUS RATH AND WILHELM CHRIST, OF OFFENBACH-ON-THE-MAIN, GERMANY, AS  
SIGNORS TO THE I. G. FARBENINDUSTRIE AKTIENGESELLSCHAFT, OF FRANK-  
FORT-ON-THE-MAIN, GERMANY.

## PROCESS OF PRODUCING MULTICOLOR EFFECTS ON VEGETABLE FIBERS AND PRODUCT THEREOF.

No Drawing. Application filed January 15, 1925, Serial No. 2,804, and in Germany February 7, 1924.

Hitherto it was not possible to produce multi-color effects or combined shades in colored textile fabrics or one-color cotton goods by superimposing vat dyestuffs on portions of said fabrics or goods previously dyed with azodyestuffs.

Now we have found that such azodyestuffs as are resistant to the action of boiling dilute caustic soda solution in the presence of cellulose, that is fast to kier-boiling, can be given a superimposed printing or dyeing with vat dyestuffs without damage to the underlying primary dyeing. In this manner multi-color effects and combined shades of an excellent fastness may be obtained.

Taking into consideration the well known instability of azodyestuffs against an alkaline hydrosulfite solution the possibility of such a dyeing method is very surprising.

As azodyestuffs we may use for this process especially the insoluble azodyestuffs produced by development on the fiber, so far as their colorings are fast to boiling caustic soda solution or kier-boiling, such as for example the combinations with the arylamides of 2,3-oxynaphthoic acid, as described in the U. S. A. Letters Patent No. 1,034,853, dated Aug. 6, 1912, and in the later publications, based on this fundamental patent, or the dyestuffs, derived from acylacetylamines, as described in the U. S. A. Letters Patents No. 1,505,568 and 1,505,569, both dated June 10, 1924, and the U. S. A. application of Arthur Zitscher, Serial No. 641,510, filed May 25, 1923, and the like.

The following examples illustrate the invention, the parts being by weight.

### Example 1.

Cotton yarn, previously dyed according to the process, described in the U. S. A. Letters Patent No. 1,099,108, dated June 2, 1914, with: 4-nitro-1,2-anisidin upon 2,3-oxynaphthoyl-beta-naphthylamin or 2,5-dichloroanilin upon 2,3-oxynaphthoyl-ortho-chloroanilin respectively and interwoven with white to colored textile fabrics, is overdyed with 0.5% (in relation to the weight of the goods) of algolbrilliantviolet R, 4 cc. of caustic soda solution of 30° Bé., 2 g. of hydrosulfite, concentrated powder, in 1 liter of liquor. Liquor: 1:10. Temperature of dyeing: 25° C. Duration of dyeing: 3/4 hour.

Bright and full red or scarlet shades on a light violet ground are obtained.

### Example 2.

Colored webs from cotton-yarn, previously dyed as in example 1 with 4-chloro-1,2-toluidin upon 2,3-oxynaphthoyl-β-naphthylamin or 5-chloro-1,2-toluidin upon 2,3-oxynaphthoyl-5-chloro-2-anisidin, and white are overcrossed with 1% of indanthrene blue G C, 20 cc. of caustic soda solution of 30° Bé., 2 g. of hydrosulfite, concentrated powder, in 1 liter of liquor. Liquor: 1:10. Temperature of dyeing: 45-60° C. Duration of dyeing: 3/4 hour.

Dark red to Bordeaux-red shades on a light blue ground result.

### Example 3.

Cotton goods, previously dyed according to the ice colors method with ortho-chloroanilin upon diacetooacetyl-ortho-tolidin (see U. S. A. Letters Patent No. 1,505,568) are overdyed with 10% of alizarine indigo 7 G, 15 cc. of caustic soda solution of 30° Bé., 3 g. of hydrosulfite, concentrated powder, in 1 liter of liquor. Liquor: 1:10. Temperature of dyeing: 85° C. Duration of dyeing: 3/4 hour.

Pure brilliant green shades are obtained. The method of padding (see U. S. A. Letters Patent No. 893,384, dated July 14, 1908) may also be used.

### Example 4.

The goods, previously dyed with ortho-chloroanilin upon diacetooacetyl-ortho-tolidin, are printed with the following printing-color and dried.

Printing-color:  
220 g. of neutral tragacanth-thickening, 95  
300 g. of gum 1:1,  
140 g. of potash,  
90 g. of glycerin,  
100 g. of rongalit C are heated, after cooling down poured into, 100  
150 g. of alizarine indigo 7 G in paste.

1000 g.

The printed goods are steamed with wet steam for 3-5 minutes in a rapid steamer-apparatus, free of air, then chromed at 106

50-60° C. (2 gr. of bichromate, 5 cc. of acetic acid of 6° Bé. in the liter), rinsed and soaped.

5 A green design upon a yellow ground is obtained.

*Example 5.*

10 Cotton yarn, previously dyed with ortho-aminoazotoluene upon diacetooacetyl-ortho-tolidin, woven with white to colored textile fabrics, is overdyed with 3% of algolbrilliantviolet R, 4 cc. of caustic soda solution of 30° Bé., 2 g. of hydrosulfite, concentrated powder, in 1 liter of liquor. Liquor: 1:10.

15 Temperature of dyeing: 50° C. Duration of dyeing:  $\frac{3}{4}$  hour.

Clear brown shades on a light violet ground are obtained.

Having now particularly described and

ascertained the nature of our said invention and in what manner the same is to be performed, we declare, that what we claim is:

1. A process of producing multi-color effects or combined shades on the vegetable fiber, consisting in superimposing vat dyestuffs on fabric portions which have been previously treated with such azodyestuffs as are resistant to the action of boiling dilute caustic soda solution in the presence of cellulose, that is, fast to kier-boiling.

2. Materials dyed or printed according to claim 1.

In testimony, that we claim the foregoing as our invention, we have signed our names, this 31st day of December, 1924.

Dr. JULIUS RATH.

Dr. WILHELM CHRIST.